

Sept. 24, 1929.

G. H. REIMER

1,729,128

IMITATION OXIDIZED SURFACE AND PROCESS THEREFOR

Filed Feb. 13, 1928



Inventor:  
George H. Reimer  
By Arthur J. Durand  
Gty.

## UNITED STATES PATENT OFFICE

GEORGE H. REIMER, OF FULTON, ILLINOIS, ASSIGNOR TO PATENT NOVELTY COMPANY,  
OF FULTON, ILLINOIS, A CORPORATION OF ILLINOIS

## IMITATION OXIDIZED SURFACE AND PROCESS THEREFOR

Application filed February 13, 1928. Serial No. 253,957.

This invention relates to processes or methods of simulating oxidized metal surfaces.

Generally stated, therefore, the object of the invention is to provide a novel and efficient process or method that will obviate the necessity of oxidizing metal, but which will produce a surface having very much the same appearance, for sheet-metal articles or other things made of metal.

10 It is also an object to provide certain details and method features tending to increase the general efficiency and the desirability of a process or method of this particular character.

15 To the foregoing and other useful ends, the invention consists in the matters hereinafter set forth and claimed, and shown in the accompanying drawings, in which the single figure is a perspective of a mail box having 20 a simulated oxidized surface produced in accordance with the principles of the invention.

The process or method comprises, for example, in the making of a mail box of the kind shown, the giving of the sheet-metal 25 box a base coat of black enamel, which may be black japan, oil varnish enamel or pyroxylin enamel, this base coat being applied to the metal surface by dipping or spraying or brushing. This base coat is then baked 30 hard, if such is required, and then afterward the black base coat is striped or spotted by applying bronze powder mixed with bronze liquid, this bronze solution being preferably sprayed on to the black base coat 35 to produce spots or stripes resembling copper or bronze or brass in appearance.

Thereafter, if greater durability is desired, a film or coat of varnish or pyroxylin lacquer is sprayed over the entire article.

40 As shown in the drawing, the result of such process or method will be dark stripes 1, if a striping effect is employed, alternating with the lighter stripes 2 of copper or bronze, the stripes preferably fading into 45 each other.

In this way, therefore, an imitation oxidized copper or other metal surface is produced, which is surprisingly handsome and effective in appearance.

50 It will be understood that the metallic

solution may be either actual metallic solution or imitation metallic solution, this being immaterial so long as the appearance of oxidized metal is produced. It will be understood, therefore, that in the claims the word "metallic" has this meaning; as it is immaterial whether metallic substances are actually employed in making the spraying solution, or whether imitation metallic materials are employed for this purpose.

Without disclaiming anything, and without prejudice to any novelty disclosed, what I claim as my invention is:

1. The method of producing an imitation oxidized metal surface, to provide an ornamental exterior simulating oxidized metal for any desired object, comprising the formation of a base coat of dark shade, and thereafter spraying a metallic solution on to the base coat in spots or stripes, leaving some of 70 the base coat exposed, and with the exposed portions of the base coat and the metallic portions fading into each other, producing the appearance of an oxidized metal surface.

2. The said method as specified in claim 75 1, the said base coat being black japan or any liquid that will produce a lustrous black surface, and the said metallic solution comprising bronze powder mixed with bronze liquid in such condition as to be easily 80 sprayed upon the black surface.

3. As an article of manufacture, an object having the desired form and having an imitation oxidized metallic surface providing an ornamental exterior simulating oxidized 85 metal formed by a base coat of lustrous dark shade, with an upper metallic coat, leaving portions of the base coat exposed, and these exposed portions fading into the metallic portions of the surface, producing the appearance of an oxidized metal surface.

4. A structure as specified in claim 3, said base coat being black japan, or any liquid that will produce a lustrous black surface, and said second mentioned coat being a dried 95 mixture of bronze powder and bronze liquid.

Specification signed this 8th day of February, 1928.

GEORGE H. REIMER.